

# UNITED STATES PATENT OFFICE.

PETER J. NAGLE, OF ROCHESTER, NEW YORK, ASSIGNOR TO CEDAROID CO. INC., OF ROCHESTER, NEW YORK, A CORPORATION.

## PAPER OR PAPER-BOARD.

1,283,422.

Specification of Letters Patent. Patented Oct. 29, 1918.

No Drawing.

Application filed November 12, 1917. Serial No. 201,464.

*To all whom it may concern:*

Be it known that I, PETER J. NAGLE, a citizen of the United States, and resident of the city of Rochester, in the county of Monroe and State of New York, have invented certain new and useful Improvements in Paper or Paper-Board, of which the following is a specification.

The present invention relates to paper or paper board, and an object of the invention is to provide a paper or paper board which, when formed into a container or receptacle of any sort, will communicate to the contents a desirable aroma. Another object of the invention is to provide a paper or paper board free from impurities and adapted to act to keep away insects or other germs from material inclosed by the paper or paper board. Still another object of the invention is to provide a paper colored to simulate cedar wood by a substance which will not affect articles inclosed by the paper, but which will, instead, impart to articles such as tobacco a desirable flavor or aroma. A still further object of the invention is to provide for incorporation within the paper a waterproofing substance which also tends to set the color when the paper is dry.

With these and other objects in view, the invention consists of the features hereinafter described and particularly pointed out in the appended claims.

Previous to this invention it has been suggested to coat and to saturate paper or paper board with substances which will act as an insecticide for articles which may be wrapped or inclosed by the paper or paper board. Not only does this necessitate the separate steps of saturating and coating the paper or paper board, but the paper or paper board must afterward be dried, which increases the cost of manufacturing the paper.

According to this invention cedar oil which is an aroma producing substance and also an insecticide is added to the paper pulp while the latter is in the digester or beater, the oil being first mixed with a suitable substance in order to form an emulsion so that it will thoroughly mix with the paper pulp. By this arrangement the oil is intimately incorporated within the paper or paper board, thus not only eliminating the coating and drying steps, but making it possible to maintain the effect of the substance within the stock for a longer time, not only because of

the intimate mixture, but because of the calendering process which occurs after the substances have been mixed with the pulp.

To form an emulsion from cedar oil the latter is mixed with sugar, so that water may be added to produce the emulsion. The emulsion may be improved if vinegar or alcohol, or both, are added to the sugar and cedar oil before the addition of water. It has also been found that the aroma of tobacco will be still further improved if licorice is added to the compound, and to this end the water which is used to produce the emulsion is first employed for dissolving powdered licorice. This licorice also acts to color the paper to simulate the color of cedar wood, and, if desired, a small amount of coloring matter, such as anilin brown, may be added to the licorice in solution. To set the color obtained from the licorice and the coloring matter, glycerin may be added to the cedar oil and sugar. This glycerin also tends to give waterproofing qualities to the paper or paper board. The sugar, in addition to producing an emulsion, tends to sweeten the tobacco inclosed by the paper. It is preferred to use the following proportions of the above-mentioned ingredients:

|           |     |    |
|-----------|-----|----|
| Water     | 25% | 85 |
| Cedar oil | 25% |    |
| Sugar     | 15% |    |
| Licorice  | 10% |    |
| Vinegar   | 10% |    |
| Alcohol   | 10% |    |
| Glycerin  | 5%  | 90 |

The compound is added slowly to the pulp, while the latter is in the beater and readily mixes with the pulp. It is preferred that the pulp shall be ground wood pulp with as few impurities as possible. The cedar oil and alcohol will kill all impurities in the pulp and the materials used in the manufacture of paper for setting the color of the paper also set the aroma of the compound, so that while the tobacco, due to the natural moisture therein, tends to absorb the compound from the paper, the latter will, at the same time, hold the compound for an indefinite time. The calendering process tends to form a surface on the paper which retards the escape of the aroma.

The paper or paper board made in accordance with this invention is especially adapted for use in or for making containers which

will communicate to their contents a desirable aroma. The specific ingredients named give a paper which is especially desirable for holding tobacco or tobacco articles, such as 5 cigars and cigarettes. The oil is so incorporated in the pulp that it is held longer than by coating or saturation. The licorice is held in the same way and at the same time acts as a coloring matter for the paper, 10 making it unnecessary to coat or line a box interiorly or exteriorly. The sugar sweetens the contents of the containers and at the same time permits the oil to be mixed with the pulp. The cedar oil and alcohol kill 15 impurities in the paper stock in the beater and the glycerin acts to water-proof the material while also setting the color. The materials used in the manufacture of the paper for setting the color of the paper also 20 set the aroma of the licorice and the cedar

oil, while permitting such aroma to be absorbed by the contents of the container.

What I claim as my invention and desire to secure by Letters Patent is:—

1. Paper containing pulp mixed with 25 cedar oil and an emulsifying agent for the cedar oil.

2. Paper containing pulp mixed with cedar oil, an emulsifying agent for cedar oil, and licorice.

3. Paper containing pulp mixed with cedar oil, sugar and licorice.

4. Paper containing pulp mixed with cedar oil, an emulsifying agent for the cedar oil, licorice, and glycerin.

5. Paper containing pulp mixed with cedar oil, an emulsifying agent for the cedar oil, licorice, and alcohol.

PETER J. NAGLE.